# EUROPEAN PATENT SPECIFICATION

(11) **EP 1 546 422 B1**
(45) Date of publication and mention of the grant of the patent: **21.02.2007**
(21) Application number: 03794565.6
(22) Date of filing: 04.09.2003
(51) Int. Cl.: C22C 1/05, C22C 27/04, C22F 1/18, B22F 3/24

(54) **METHOD OF FORMING SAG-RESISTANT MOLYBDENUM-LANTHANA ALLOYS**
VERFAHREN ZUR HERSTELLUNG VON SAG-BESTÄNDIGEN MOLYBDÄN-LANTHANOXID-LEGIERUNGEN
PROCEDE DE FORMATION D'ALLIAGES DE MOLYBDENE-OXYDE DE LANTHANE RESISTANT A L'AFFAISSEMENT

(30) Priority: 04.09.2002 US 408087 P
(43) Date of publication of application: 29.06.2005
(73) Proprietor: OSRAM SYLVANIA INC., Danvers, MA 01923 (US)
(72) Inventor: WINNICKA, Maria, B., Sayre, PA 18840 (US)
(74) Representative: Lambert, Ian Robert
(86) International application number: PCT/US2003/027439
(87) International publication number: WO 2004/022801

(56) References cited:
- US-A- 3 785 801
- US-A- 4 514 234
- US-A- 4 950 327
- US-A- 5 134 039
- US-A- 5 435 829
- US-A- 5 835 841
- US-A- 5 868 876
- US-A- 6 102 979

## Description

### TECHNICAL FIELD

This invention relates generally to methods for forming dispersion-strengthened alloys of molybdenum. More particularly, this invention relates to methods of forming molybdenum-lanthana alloys having sag-resistant microstructures.

### BACKGROUND OF THE INVENTION

Molybdenum alloys which have been dispersion-strengthened with particles of lanthanum oxide (lanthana), La₂O₃, are desirable for use in high temperature applications because of their high melting point and good mechanical properties at high temperatures, in particular, resistance to sag and creep. The alloys are formed by combining molybdenum powder with from about 0.1 to about 5 weight percent (wt.%) of lanthanum oxide powder or an equivalent amount of a lanthanum oxide precursor, such as La(OH)₃ or La(NO₃)₃, which is then converted to the oxide by heating. The size of the lanthanum oxide particles dispersed in the molybdenum matrix is generally preferred to be less than about 1 µm, however, the particles may be as large 5-10 µm. After compacting and sintering, the sintered body is deformed by mechanical working, e.g., rolling, swaging, drawing, or hammering, and then is then recrystallized to generate the desired microstructure. For sag and creep resistance, the preferred microstructure consists of large, interlocking grains which are elongated in the direction of the applied mechanical work.

The recrystallization behavior of the alloy is affected by the prior amount of deformation. When the undeformed or fully recrystallized alloy is being cold worked, the density of dislocations within the alloy increases. This occurs first at the grain boundaries and then progresses further into the bulk of the grains as the amount of cold work increases. Prior art methods have employed high degrees of deformation (>60%) in order to achieve high-temperature strength and creep-resistance.

Japanese Patent Publication 59-177345 (1984) describes a molybdenum-lanthana alloy for structural purposes. The alloy has a high secondary recrystallization temperature and high high-temperature strength. The alloy contains 1 to 5 wt.% lanthana (La₂O₃) particles having an average size of not more than 3 µm which are uniformly dispersed in molybdenum. For structural purposes, the material is preferably worked from the sinter by a working factor of at least 60% and then heated above the secondary recrystallization temperature.

U.S. Patent No. 4,950,327 to Eck et al. (1990) describes a high-temperature, creep-resistant molybdenum-lanthana alloy having a tiered structural arrangement. After sintering, the alloy is mechanically reformed in gradations of about 10% without heating the alloy above its recrystallization temperature. Once the degree of reforming is at least 85%, the alloy is finally subjected to a recrystallization anneal.

U.S. Patent No. 4,514,234 discloses a process of manufacturing a doped molybdenum board in which a preliminary area reduction working at a working ratio between 45 and 85% is performed, followed by a preliminary recrystallization. Another area reduction working is performed at a total working ratio which is not less than 85%, and the thus treated sintered ingot is subjected to a final recrystallization annealing step. The molybdenum sintered ingot may contain inter alia 1 weight % of La₂O₃.

One disadvantage with the prior art methods is that the dimensions of the feed material must be substantially greater than the dimensions of the finally recrystallized material in order to impart the required high degree of deformation. This leads to less flexibility in the manufacturing process. Another disadvantage is that the large amount of stored energy in the material caused by the high degree of deformation can lead to spontaneous grain growth in the material during recrystallization. This may make it more difficult to control grain size in the finally recrystallized material.

### SUMMARY OF THE INVENTION

It has been discovered that a sag-resistant microstructure can be obtained in a molybdenum-lanthana alloy using a degree of deformation of from 7% to 18%. As used herein, the degree of deformation refers to the percentage reduction in at least one dimension of the feed material, e.g., sheet thickness. Preferably, the degree of deformation is from 12% to 17%. The alloy may be deformed directly from the as-sintered state to its finished form and then finally recrystallized or, preferably, the alloy can worked from the as-sintered state to a near-finished form, recrystallized, and then deformed to its finished form and finally recrystallized. Preferably, the recrystallization of the alloy in its near-finished form is conducted at a temperature of from 1150°C to 1400°C. The final recrystallization is preferably conducted at about 1900°C. Preferably, the amount of lanthana in the alloy ranges from 0.4 wt.% to 1.0 wt.%, more preferably, from 0.6 wt.% to 0.7 wt.%.

The grain size after final recrystallization is larger because the predominant mechanism occurring during the heat treatment is the annihilation of dislocations at the neighboring grain boundaries causing some grain boundaries to disappear. This is generally referred to as strain-induced grain boundary migration. After final recrystallization, the grains tend to exhibit less elongation than grains resulting from methods which use high degrees of deformation. Typically, the aspect ratio for the grains produced by the method of this invention is no more than 4:1. Also, since the degree of reformation needed to produce the sag-resistant microstructure is 18% or less, the feed material need not be much larger than the finished product and there is a greater potential to control grain size in the finished material because of the lower amount of stored energy in the material prior to final recrystallization. Hence, the method of this invention is more flexible for manufacturers of refractory metal products.

### BRIEF DESCRIPTION OF THE DRAWINGS

Fig. 1A is a photomicrograph of the microstructure of the molybdenum-lanthana alloy of Example 1 after recrystallization and rolling to 0.15 cm thickness.
Fig. 1B is a photomicrograph of sag-resistant microstructure of the molybdenum-lanthana alloy of Example 1 after final recrystallization.
Fig. 2A is a photomicrograph of the microstructure of the molybdenum-lanthana alloy of Example 2 after recrystallization and rolling to 0.10 cm thickness.
Fig. 2B is a photomicrograph of sag-resistant microstructure of the molybdenum-lanthana alloy of Example 2 after final recrystallization.

### DETAILED DESCRIPTION OF THE INVENTION

For a better understanding of the present invention, together with other and further objects, advantages and capabilities thereof, reference is made to the following disclosure and appended claims taken in conjunction with the above-described drawings.

### EXAMPLE 1

Pure molybdenum metal powder with grain size of 3.5 µm was mixed with 0.7 weight percent (wt.%) of La(OH)₃ powder having a grain size of 0.65 µm. The mixture was isostatically pressed at 240 MPa to form a pressed slab with dimensions of 64 cm x 38 cm x 5 cm. The slab was subsequently rolled at varying temperatures; starting at 980°C, followed by 785°C, and finally at ambient temperature to a thickness of 0.17 cm. The sheet was then recrystallized at 1400°C and then rolled at ambient temperature to the thickness of 0.15 cm, (about 12% deformation). The microstructure of the recrystallized and rolled sheet is shown in Fig. 1A. The rolled sheet was subjected to a final recrystallization anneal at 1900°C to produce the sag-resistant microstructure which is shown in Fig. 1B.

### Example 2

Pure molybdenum metal powder with grain size of 3.5 µm was mixed with 0.7 wt.% La(OH)₃ powder with a grain size of 0.65 µm. The mixture was isostatically pressed at 240 MPa to form a pressed slab with dimensions of 64 cm x 38 cm x 5 cm. The slab was subsequently rolled at varying temperatures; starting at 980°C, followed by 785°C, and finally at ambient temperature to a thickness of 0.12 cm. The sheet was then recrystallized at 1150°C. Subsequently it was rolled at ambient temperature to the thickness of 0.10 cm (about 17% deformation). The microstructure of the recrystallized and rolled sheet is shown in Fig. 2A. Upon a final recrystallization anneal at 1900°C, the sheet material exhibited the sag-resistant microstructure shown in Fig. 2B.

The sag resistance of 0.5 in. x 5.6 in. samples of the sag-resistant molybdenum-lanthana sheet material from Examples 1 and 2 was measured according to the following procedure. The samples were supported at opposite ends and a 10 g weight placed on the sample at the center point between the supports. The distance between the supports was 4.2 inches. At the start of the test, the distance between the reference plate and the 0.15-cm-thick sample was 0.5 in. at the point directly below the 10-g load. The corresponding distance for the 0.10-cm-thick sample was 0.4375 in. at the start of the test. Sag was measured as the amount of deflection of the sample toward the reference plate after heating the sample at 1900°C for 1 hour. Six such heating cycles were carried out for each sample and the amount of deflection measured after each cycle. The cumulative amount of deflection is reported in the following table. The sag resistance of the materials was found to be equivalent to commercially available non-sag molybdenum-lanthana sheet material.

**Table**

| **Material Thickness** | **Width (in.)** | **Length (in.)** | **Center Load (g)** | **Total Sag (in.)** |
|---|---|---|---|---|
| 0.15 cm | 0.5 | 5.6 | 9.99 | 0.0625 |
| 0.10 cm | 0.5 | 5.6 | 9.98 | 0.0313 |

## Claims

1. A method for forming a sag-resistant molybdenum-lanthana alloy comprising:
(a) forming a sintered body of a molybdenum-lanthana alloy wherein the alloy contains from 0.1 weight percent to 5 weight percent lanthana;
(b) mechanically working the sintered body to a near-finished form;
(c) recrystallizing the sintered body in its near-finished form;
(d) mechanically deforming the recrystallized, sintered body to a finished form wherein the degree of deformation is from 7% to 18%; and
(e) subjecting the sintered body in its finished form to a final recrystallization annealing.

2. The method of claim 1 wherein the degree of deformation is from 12% to 17%.

3. The method of claim 1 wherein the final recrystallization annealing is performed at about 1900°C.

4. The method of claim 1 wherein the sintered body in its near-finished form is recrystallized at a temperature from 1150°C to 1400°C.

5. The method of claim 1 wherein the molybdenum-lanthana alloy contains from 0.4 weight percent to 1.0 weight percent lanthana.

6. The method of claim 1 wherein the sintered body is subjected to one or more heat treatments during the mechanical working in step (b).

7. The method of claim 3 wherein the molybdenum-lanthana alloy contains from 0.6 weight percent to 0.7 weight percent lanthana.

8. The method of claim 1 wherein: the molybdenum-lanthana alloy contains from 0.4 weight percent to 1.0 weight percent lanthana; the sintered body in its near-finished form is recrystallized at a temperature from 1150°C to 1400°C; and the final recrystallization annealing is performed at about 1900°C.

9. The method of claim 8 wherein the degree of deformation is from 12% to 17%.

10. The method of claim 8 wherein the molybdenum-lanthana alloy contains from 0.6 weight percent to 0.7 weight percent lanthana.

11. A method for forming a sag-resistant molybdenum-lanthana alloy comprising:
(a) forming a sintered body of a molybdenum-lanthana alloy wherein the alloy contains from 0.1 weight percent to 5 weight percent lanthana;
(b) mechanically deforming the sintered body directly from the as-sintered state to a finished form wherein the degree of deformation is from 7% to 18%; and
(c) subjecting the sintered body in its finished form to a final recrystallization annealing.

12. The method of claim 11 wherein the degree of deformation is from 12% to 17%.

13. The method of claim 11 wherein the final recrystallization annealing is performed at about 1900°C.

14. The method of claim 11 wherein the molybdenum-lanthana alloy contains from 0.4 weight percent to 1.0 weight percent lanthana.

15. The method of claim 11 wherein the molybdenum-lanthana alloy contains from 0.6 weight percent to 0.7 weight percent lanthana.

16. The method of claim 13 wherein the degree of deformation is from 12% to 17%.

17. The method of claim 16 wherein the molybdenum-lanthana alloy contains from 0.6 weight percent to 0.7 weight percent lanthana.

## Patentansprüche

1. Verfahren zur Herstellung einer durchbiegungsbeständigen Molybdän-Lanthanoxid-Legierung, umfassend:
(a) Bilden eines Sinterkörpers aus einer Molybdän-Lanthanoxid-Legierung, wobei die Legierung 0,1 Gew.-% bis 5 Gew.-% Lanthanoxid enthält,
(b) mechanisches Umformen des Sinterkörpers in eine nahezu fertiggestellte Form,
(c) Rekristallisieren des Sinterkörpers in seiner nahezu fertiggestellten Form,
(d) mechanisches Verformen des rekristallisierten Sinterkörpers in eine fertiggestellte Form, wobei der Grad der Verformung 7 % bis 18 % beträgt, und
(e) Unterziehen des Sinterkörpers in seiner fertiggestellten Form einem abschließenden Rekristallisationsanlassen.

2. Verfahren nach Anspruch 1, bei dem der Grad der Verformung 12 % bis 17 % beträgt.

3. Verfahren nach Anspruch 1, bei dem das abschließende Rekristallisationsanlassen bei etwa 1900°C durchgeführt wird.

4. Verfahren nach Anspruch 1, bei dem der Sinterkörper in seiner nahezu fertiggestellten Form bei einer Temperatur von 1150°C bis 1400°C rekristallisiert wird.

5. Verfahren nach Anspruch 1, bei dem die Molybdän-Lanthanoxid-Legierung 0,4 Gew.-% bis 1,0 Gew.-% Lanthanoxid enthält.

6. Verfahren nach Anspruch 1, bei dem der Sinterkörper während des mechanischen Umformens im Schritt (b) einer oder mehreren Wärmebehandlung(en) unterzogen wird.

7. Verfahren nach Anspruch 3, bei dem die Molybdän-Lanthanoxid-Legierung 0,6 Gew.-% bis 0,7 Gew.-% Lanthanoxid enthält.

8. Verfahren nach Anspruch 1, bei dem die Molybdän-Lanthanoxid-Legierung 0,4 Gew.-% bis 1,0 Gew.-% Lanthanoxid enthält, der Sinterkörper in seiner nahezu fertiggestellten Form bei einer Temperatur von 1150°C bis 1400°C rekristallisiert wird, und das abschließende Rekristallisationsanlassen bei etwa 1900°C durchgeführt wird.

9. Verfahren nach Anspruch 8, bei dem der Verformungsgrad 12 % bis 17 % beträgt.

10. Verfahren nach Anspruch 8, bei dem die Molybdän-Lanthanoxid-Legierung 0,6 Gew.-% bis 0,7 Gew.-% Lanthanoxid enthält.

11. Verfahren zur Herstellung einer durchbiegungsbeständigen Molybdän-Lanthanoxid-Legierung, umfassend:
(a) Bilden eines Sinterkörpers aus einer Molybdän-Lanthanoxid-Legierung, wobei die Legierung 0,1 Gew.-% bis 5 Gew.-% Lanthanoxid enthält,
(b) mechanisches Verformen des Sinterkörpers direkt ausgehend von dem Zustand nach dem Sintern zu einer fertiggestellten Form, wobei der Grad der Verformung 7 % bis 18 % beträgt, und
(c) Unterziehen des Sinterkörpers in seiner fertiggestellten Form einem abschließenden Rekristallisationsanlassen.

12. Verfahren nach Anspruch 11, bei dem der Grad der Verformung 12 % bis 17 % beträgt.

13. Verfahren nach Anspruch 11, bei dem das abschließende Rekristallisationsanlassen bei etwa 1900°C durchgeführt wird.

14. Verfahren nach Anspruch 11, bei dem die Molybdän-Lanthanoxid-Legierung 0,4 Gew.-% bis 1,0 Gew.-% Lanthanoxid enthält.

15. Verfahren nach Anspruch 11, bei dem die Molybdän-Lanthanoxid-Legierung 0,6 Gew.-% bis 0,7 Gew.-% Lanthanoxid enthält.

16. Verfahren nach Anspruch 13, bei dem der Verformungsgrad 12 % bis 17 % beträgt.

17. Verfahren nach Anspruch 16, bei dem die Molybdän-Lanthanoxid-Legierung 0,6 Gew.-% bis 0,7 Gew.-% Lanthanoxid enthält.

## Revendications

1. - Procédé de formation d'un alliage de molybdène-oxyde de lanthane résistant à l'affaissement comprenant les opérations consistant à :
(a) former un corps fritté d'un alliage de molybdène-oxyde de lanthane, l'alliage contenant de 0,1 pour cent en poids à 5 pour cent en poids d'oxyde de lanthane ;
(b) travailler mécaniquement le corps fritté jusqu'à une forme quasi-finie ;
(c) recristalliser le corps fritté dans sa forme quasi-finie ;
(d) déformer mécaniquement le corps fritté, recristallisé, jusqu'à une forme finie, le degré de déformation étant de 7% à 18% ; et
(e) soumettre le corps fritté dans sa forme finie à un recuit de recristallisation final.

2. - Procédé selon la revendication 1, dans lequel le degré de déformation est de 12% à 17%.

3. - Procédé selon la revendication 1, dans lequel le recuit de recristallisation final est effectué à environ 1900°C.

4. - Procédé selon la revendication 1, dans lequel le corps fritté dans sa forme presque finie est recristallisé à une température de 1150°C à 1400°C.

5. - Procédé selon la revendication 1, dans lequel l'alliage de molybdène-oxyde de lanthane contient de 0,4 pour cent en poids à 1,0 pour cent en poids d'oxyde de lanthane.

6. - Procédé selon la revendication 1, dans lequel le corps fritté est soumis à un ou plusieurs traitements thermiques pendant le travail mécanique dans l'étape (b).

7. - Procédé selon la revendication 3, dans lequel l'alliage de molybdène-oxyde de lanthane contient de 0,6 pour cent en poids à 0,7 pour cent en poids d'oxyde de lanthane.

8. - Procédé selon la revendication 1, dans lequel : l'alliage de molybdène-oxyde de lanthane contient de 0,4 pour cent en poids à 1,0 pour cent en poids d'oxyde de lanthane ; le corps fritté dans sa forme quasi-finie est recristallisé à une température de 1150°C à 1400°C ; et le recuit de recristallisation final est effectué à environ 1900°C.

9. - Procédé selon la revendication 8, dans lequel le degré de déformation est de 12% à 17%.

10. - Procédé selon la revendication 8, dans lequel l'alliage de molybdène-oxyde de lanthane contient de 0,6 pour cent en poids à 0,7 pour cent en poids d'oxyde de lanthane.

11. - Procédé de formation d'un alliage de molybdène-oxyde de lanthane résistant à l'affaissement comprenant les opérations consistant à :
(a) former un corps fritté d'un alliage de molybdène-oxyde de lanthane, l'alliage contenant de 0,1 pour cent en poids à 5 pour cent en poids d'oxyde de lanthane ;
(b) déformer mécaniquement le corps fritté directement de l'état tel que fritté à une forme finie, le degré de déformation étant de 7% à 18% ; et
(c) soumettre le corps fritté dans sa forme finie à un recuit de recristallisation final.

12. - Procédé selon la revendication 11, dans lequel le degré de déformation est de 12% à 17%.

13. - Procédé selon la revendication 11, dans lequel le recuit de recristallisation final est effectué à environ 1900°C.

14. - Procédé selon la revendication 11, dans lequel l'alliage de molybdène-oxyde de lanthane contient de 0,4 pour cent en poids à 1,0 pour cent en poids d'oxyde de lanthane.

15. - Procédé selon la revendication 11, dans lequel l'alliage de molybdène-oxyde de lanthane contient de 0,6 pour cent en poids à 0,7 pour cent en poids d'oxyde de lanthane.

16. - Procédé selon la revendication 13, dans lequel le degré de déformation est de 12% à 17%.

17. - Procédé selon la revendication 16, dans lequel l'alliage de molybdène-oxyde de lanthane contient de 0,6 pour cent en poids à 0,7 pour cent en poids d'oxyde de lanthane.
